



US007780496B2

(12) **United States Patent**  
**Liu et al.**

(10) **Patent No.:** **US 7,780,496 B2**  
(45) **Date of Patent:** **Aug. 24, 2010**

(54) **METHOD FOR FABRICATING ELECTRON Emitter**

(75) Inventors: **Peng Liu**, Beijing (CN); **Shou-Shan Fan**, Beijing (CN); **Liang Liu**, Beijing (CN); **Kai-Li Jiang**, Beijing (CN)

(73) Assignees: **Tsinghua University**, Beijing (CN); **Hon Hai Precision Industry Co., Ltd.**, Tu-Cheng, Taipei Hsien (TW)

(\*) Notice: Subject to any disclaimer, the term of this patent is extended or adjusted under 35 U.S.C. 154(b) by 270 days.

(21) Appl. No.: **11/986,851**

(22) Filed: **Nov. 26, 2007**

(65) **Prior Publication Data**

US 2008/0227360 A1 Sep. 18, 2008

(30) **Foreign Application Priority Data**

Nov. 24, 2006 (CN) 2006 1 0157040

(51) **Int. Cl.**

*H01J 9/04* (2006.01)  
*H01J 1/02* (2006.01)  
*H01J 1/00* (2006.01)  
*H01J 9/02* (2006.01)  
*H01J 63/02* (2006.01)

(52) **U.S. Cl.** 445/50; 445/51; 313/309; 313/310; 313/311; 313/495

(58) **Field of Classification Search** 445/50, 445/51, 24; 313/309–311, 495

See application file for complete search history.

(56) **References Cited**

U.S. PATENT DOCUMENTS

4,940,916 A 7/1990 Borel et al.  
5,945,777 A 8/1999 Janning et al.

5,986,389 A \* 11/1999 Tsukamoto ..... 313/310  
6,366,015 B1 \* 4/2002 Shibata ..... 313/495  
6,630,772 B1 \* 10/2003 Bower et al. ..... 313/311  
7,065,857 B2 \* 6/2006 Watanabe et al. ..... 29/592.1  
7,252,749 B2 \* 8/2007 Zhou et al. ..... 204/484  
7,375,460 B2 \* 5/2008 Ishizuka et al. ..... 313/495  
7,455,757 B2 \* 11/2008 Oh et al. ..... 204/490  
2002/0060514 A1 5/2002 Nakamoto  
2003/0085650 A1 \* 5/2003 Cathey et al. ..... 313/495  
2004/0095050 A1 5/2004 Liu et al.  
2006/0073089 A1 \* 4/2006 Ajayan et al. ..... 423/447.2  
2006/0097615 A1 5/2006 Tsakalakos et al.  
2006/0108906 A1 \* 5/2006 Gosain et al. ..... 313/309  
2007/0063633 A1 3/2007 Yokota et al.  
2007/0144780 A1 6/2007 Jiang et al.

(Continued)

FOREIGN PATENT DOCUMENTS

CN 1433039 A 7/2003

(Continued)

*Primary Examiner*—Karabi Guharay

*Assistant Examiner*—Sheryl Hull

(74) *Attorney, Agent, or Firm*—Jeffrey T. Knapp

(57) **ABSTRACT**

A method for fabricating a surface-conduction electron emitter includes the steps of: (a) providing a substrate; (b) disposing two lower layers on the surface of the substrate, the two lower layers are parallel and apart from each other; (c) disposing a plurality of carbon nanotube elements on the lower layers; (d) disposing two upper layers on the two lower layers, and thereby, sandwiching the carbon nanotube elements therebetween; and (e) forming a micro-fissure between the carbon nanotube elements.

**20 Claims, 14 Drawing Sheets**

20



U.S. PATENT DOCUMENTS

2007/0145878 A1 6/2007 Liu et al.  
2009/0045720 A1\* 2/2009 Lee et al. .... 313/503

JP 2003-45366 2/2003

JP 2005162571 6/2005

JP 2007-128892 5/2007

JP 2007-173238 7/2007

KR 2003014904 A \* 2/2003

KR 20030014904 2/2003

TW 200302499 A 8/2003

TW I257413 7/2006

FOREIGN PATENT DOCUMENTS

CN 1790598 6/2006  
JP 2001-52598 2/2001  
JP 2002-157951 5/2002

\* cited by examiner



FIG. 1  
(PRIOR ART)



FIG. 2



FIG. 3



FIG. 4



FIG. 5



FIG. 6



FIG. 7



FIG. 8



FIG. 9



FIG. 10



FIG. 11



FIG. 12



FIG. 13



FIG. 14

## 1

METHOD FOR FABRICATING ELECTRON  
EMITTER

## RELATED APPLICATIONS

This application is related to commonly-assigned applications entitled, "SURFACE-CONDUCTION ELECTRON EMITTER", filed Nov. 26, 2007, Ser. No. 11/986,850. Disclosure of the above-identified application is incorporated herein by reference.

## BACKGROUND

## 1. Field of the Invention

The invention relates generally to methods for fabricating electron emitters and, particularly, to a method for fabricating a surface-conduction electron emitter.

## 2. Discussion of Related Art

Recently, development of flat panel displays (FPDs) has increased. Flat panel displays include field emission displays (FED), liquid crystal displays (LCD), plasma display panels (PDP), etc.

Among the various types of flat panel displays, liquid crystal displays are extensively investigated, but LCDs still have problems such as low brightness and narrow viewing angle when compared with the other FPDs. For plasma display panels, high energy consumption and low color fidelity are the main obstacles.

For the field emission display panels, the most developed display type is the "Spindt" type field emission display, which typically includes a plurality of micro-tip structures. However, the fabrication cost of the micro-tip structures is high and they are difficulties in increasing the size of the display.

A recently developed field emission display is a surface-conduction electron emitter display (SED) with a plurality of surface-conduction electron emitters (SCEs) therein. In the SCE, electrons are emitted from a micro-fissure in a low work function material, such as diamond or palladium oxide (PdO). The surface-conduction electron emitter display, typically, uses one surface-conduction electron emitter per pixel. The micro-fissure, which may be only a few nanometers wide, emits electrons upon electrical stimulation. FIG. 1 shows a prior art of a surface-conduction electron emitter 10 including a cathode 12 and an anode 14 with a fluorescent layer 16 formed thereon. The cathode 12 includes a substrate 110, two electrodes 112 and 114, a conductive film 116 with a gap formed thereon, and a deposit layer 118 disposed in the gap of the conductive film 116. A nanometer scale micro-fissure 120 is formed in the middle of the deposit layer 118. In use, a voltage is applied to the two electrodes 112 and 114. Due to an electron tunneling effect, electrons emitted from the electrode 112 are transmitted to the electrode 114. An accelerating voltage is applied to the anode 14. Thus, electrons are partially deviated from the transmitting direction to the anode 14, and the fluorescent layer 16 can be excited to produce a visible light.

The low work function materials used in the surface-conduction electron emitter can be simply deposited into the gap between the electrodes by using ink-jet printing. Therefore, the method for fabricating the SED is simple and the cost is low. In a conventional 40-inch SED, the contrast is about 8600:1, the thickness is about 10 millimeters, and the power used is only half that used by a same sized LCD.

However, in the above-described surface-conduction electron emitters, the micro-fissures are generally formed using high current for a long period of time. Therefore, a large amount of energy is needed during fabrication of the surface-

## 2

conduction electron emitters. Additionally, because the width of the micro-fissure is only several nanometers, a portion of the electrons emitted from one electrode reach the other electrode before the accelerating voltage can deflect them from their path. Thus, the efficiency of the surface-conduction electron emitters is relatively low.

What is needed, therefore, is to provide a method for fabricating an electron emitter that is simple, and the efficiency of the electron emitter is increased.

10

## SUMMARY

In one embodiment, a method for fabricating a surface-conduction electron emitter includes the steps of: (a) providing a substrate; (b) disposing two lower layers on the surface of the substrate, the two lower layers are parallel and apart from each other; (c) disposing a plurality of carbon nanotube elements on the lower layers; (d) disposing two upper layers on the two lower layers, and thereby, sandwiching the carbon nanotube elements therebetween; and (e) forming a micro-fissure between adjacent carbon nanotube elements.

Other advantages and novel features of the present method for fabricating an electron emitter will become more apparent from the following detailed description of preferred embodiments when taken in conjunction with the accompanying drawings.

## BRIEF DESCRIPTION OF THE DRAWINGS

30 Many aspects of the present invention of the method for fabricating an electron emitter can be better understood with reference to the following drawings.

FIG. 1 is a side view of a conventional surface-conduction electron emitter;

35 FIG. 2 is a cross-section view of a surface-conduction electron emitter, in accordance with a first embodiment;

FIG. 3 and FIG. 4 are top views of the surface-conduction electron emitter of FIG. 2;

40 FIG. 5 is a side view of an electron source including the surface-conduction electron emitter of FIG. 2;

FIG. 6 is a cross-section of a surface-conduction electron emitter, in accordance with a second embodiment;

FIG. 7 is a cross-section of a surface-conduction electron emitter, in accordance with a third embodiment;

45 FIG. 8 is a cross-section view of a surface-conduction electron emitter, in accordance with a fourth embodiment;

FIG. 9 shows a Scanning Electron Microscope (SEM) image of a top view of the surface-conduction electron emitter of FIG. 2.

50 FIG. 10 is a flow chart of a method for fabricating the surface-conduction electron emitter, in accordance with the first embodiment; and

FIG. 11 to FIG. 14 are schematic views of the method of FIG. 10.

55 Corresponding reference characters indicate corresponding parts throughout the several views. The exemplifications set out herein illustrate at least one preferred embodiment of the present method for fabricating an electron emitter, in at least one form, and such exemplifications are not to be construed as limiting the scope of the invention in any manner.

DETAILED DESCRIPTION OF PREFERRED  
EMBODIMENTS

60 Reference will now be made to the drawings to describe, in detail, embodiments of the present method for fabricating an electron emitter.

Referring to FIG. 2, a surface-conduction electron emitter 20 in the first embodiment includes a substrate 22, a first electrode 24, a second electrode 24', and two line-shaped carbon nanotube elements 26. The first electrode 24 and the second electrode 24' are parallel to each other and disposed on the substrate 22.

The first electrode 24 and the second electrode 24' respectively include lower layers 242 and 242', and upper layers 244 and 244'. The lower layers 242 and 242' are disposed on a surface of the substrate 22. The upper layers 244 and 244' are disposed on the lower layers 242 and 242'. Two carbon nanotube elements 26 are respectively sandwiched by the upper layers 244 and 244' and the lower layers 242 and 242', and thereby, fixed on the first electrode 24 and the second electrode 24'. Each carbon nanotube element 26 includes at least one emitting end 262 protruding from the first electrode 24 and/or the second electrode 24'. The emitting ends 262 of the two carbon nanotube elements 26 are opposite to each other. A micro-fissure 28 is formed between the two opposite emitting ends 262 of the carbon nanotube elements 26.

The substrate 22 can, beneficially, be made of an insulative material selected from a group consisting of quartz, glass, ceramic, and plastic, or of a conductive material, with an insulative layer covered thereon. The insulative layer can, usefully, be an oxide layer. The thickness of the substrate 22 is dependent on the actual need/use. In the first embodiment, the substrate 22 is made of a silicon wafer with a silicon dioxide layer formed thereon. The thickness of the silicon dioxide layer is in the approximate range from 0.5 to 1 micron.

The carbon nanotube element 26 can, advantageously, include at least one material selected from a group consisting of carbon nanotubes and carbon nanotube bundles. The carbon nanotube bundles include a plurality of carbon nanotubes joined end to end.

The first electrode 24 and the second electrode 24' can, opportunely, be made of a metallic material such as titanium (Ti), platinum (Pt), or gold, silver, copper, or alloys thereof. The thickness of the first electrode 24 and the second electrode 24' are in the approximate range from 20 to 150 nanometers. The width of the first electrode 24 and the second electrode 24' are in the approximate range from several microns to several tens of microns. The length of the first electrode 24 and the second electrode 24' is dependent on the actual needs/use. The width of the micro-fissure 28 is in the approximate range from several microns to several hundreds of microns. Quite suitably, in the first embodiment, the width of the first electrode 24 and the second electrode 24' are in the approximate range from 90 to 190 microns. The width of the micro-fissure 28 is about 10 microns.

The lower layers 242 and 242' can, opportunely, be made of a metallic material with a high adhesion force such as titanium (Ti), tungsten (W), or chromium (Cr) to enhance the adhesion force between the lower layers 242 and 242' and the substrate 22. The upper layers 244 and 244' can, beneficially, be made of a metallic material with high conductivity such as gold, platinum (Pt) or palladium (Pd) to enhance electrical contact and reduce resistance between the upper layers 244 and 244' and the carbon nanotube elements 26. Further, the lower layers 242 and 242' can include a plurality of metallic layers. The lower layer contacted with the substrate 22 can, advantageously, be made of a metallic material with high friction coefficient such as titanium (Ti), tungsten (W), or chromium (Cr). The upper layer contacted with the carbon nanotube elements 26 can, rather appropriately, be made of a metallic material with high conductivity such as gold, platinum (Pt) or palladium (Pd).

It is to be understood that, in the first embodiment, a plurality of carbon nanotube elements 26 can, beneficially, be sandwiched by the first electrode 24 and/or the second electrode 24', and thereby, be fixed thereon. Further, a plurality of carbon nanotube elements 26 are parallel to each other and the substrate 22. Referring to FIG. 3, a plurality of the carbon nanotube elements 26 can be sandwiched by the first electrode 24, only. Each carbon nanotube element 26 includes at least one emitting end 262 protruding from the first electrode 24. The at least one emitting end 262 points to the second electrode 24'. The micro-fissure 28 is, thereby, formed between the at least one emitting end 262 and the second electrode 24'. Referring to FIG. 4, a plurality of the carbon nanotube elements 26 can, rather appropriately, be respectively sandwiched by the first electrode 24 and the second electrode 24'. The carbon nanotube elements 26 include at least one emitting end 262 in each electrode. The emitting ends 262 of the first electrode 24 and the second electrode 24' are opposite to each other. The micro-fissure 28 is, thereby, formed between the opposite emitting ends 262 of the first electrode 24 and the second electrode 24'.

It will be apparent to those having ordinary skill in the field of the present invention that the first electrode 24 and/or the second electrode 24' can be integrally formed. Beneficially, the carbon nanotube elements 26 can be directly fixed on the surfaces of the first electrode 24 and/or the second electrode 24' by using a conductive glue/adhesive or be embedded in the first electrode 24 and/or the second electrode 24'.

Referring to FIG. 5, in the first embodiment, an electron source 30 is further provided. The electron source includes a plurality of the above-described surface-conduction electron emitters 20. Pairs of the first electrodes 24 and the second electrodes 24' are disposed on the same substrate 22 parallel to each other. A plurality of the carbon nanotube elements 26 are fixed on the first electrodes 24 and the second electrodes 24'. Each carbon nanotube element 26 includes at least one emitting end 262 protruding from the electrode. The micro-fissures 28 are formed between two opposite emitting ends 262. It is to be understood that the carbon nanotube elements 26 can be fixed on the first electrodes 24 or the second electrodes 24' only. Further, the micro-fissures 28 can be formed between the emitting ends 262 and the second electrodes 24' or the first electrodes 24. The electron source 30 can be used in a SED. The SED includes an electron source 30, an anode 32 disposed above the electron source 30, and a fluorescent layer 34 formed on the anode 32. In use, a voltage is applied to the first electrode 24 and the second electrode 24'. Due to the excellent field emission property of the carbon nanotubes, electrons are able to emit from the carbon nanotube element 26 of the second electrode 24' and move toward the first electrode 24. An accelerating voltage is applied on the anode 32, and accordingly, the electrons deviate from their path and reach the anode 32. When the electrons collide against the fluorescent layer 34, a visible light is produced. In the first embodiment, when the accelerating voltage and the voltage between the first electrode 24 and the second electrode 24' is in a ratio of about 6:1, the anode current is the same as the current between the first electrode 24 and the second electrode 24'. As a result, a relatively high efficiency of the electron source 30 can be achieved.

Referring to FIG. 6, the surface-conduction electron emitter 40 in the second embodiment is similar to the surface-conduction electron emitter 20 in the first embodiment, and includes a substrate 42, a first electrode 44, a second electrode 44', and two carbon nanotube elements 46. The first electrode 44 and the second electrode 44' are parallel to each other and disposed on the substrate 42.

The first electrode 44 and the second electrode 44' respectively include lower layers 442 and 442', and upper layers 444 and 444'. The lower layers 442 and 442' are disposed on the surface of the substrate 42. The upper layers 444 and 444' are disposed on the lower layers 442 and 442'. Two carbon nanotube elements 46 are respectively sandwiched by the upper layers 444 and 444' and the lower layers 442 and 442', and thereby, fixed on the first electrode 44 and the second electrode 44'. Each carbon nanotube element 46 includes at least one emitting end protruding from the first electrode 44 and/or the second electrode 44'. Two emitting ends of the two carbon nanotube elements 46 are opposite to each other. A micro-fissure is formed between the two opposite emitting ends of the carbon nanotube elements 46. A spacer 48 is further disposed on the surface of the substrate 42, between the first electrode 44 and the second electrode 44'.

The thickness of the spacer 48 is less than or equal to the thickness of the lower layers 442 and 442'. The spacer 48 can, beneficially, be made of a material selected from a group consisting of silicon dioxide, alumina, metal oxides, and ceramic. In the second embodiment, the spacer 48 is a layer of silicon dioxide. The thickness of the spacer 48 is in the approximate range from 40 to 70 nanometers. The spacer 48 can prevent a bend or a break of the carbon nanotube elements 40 protruding from the first electrodes 44 and the second electrodes 44' that could be caused by the effects of gravity or the electrical field.

Referring to FIG. 7, the surface-conduction electron emitter 50 in the third embodiment is similar to the surface-conduction electron emitter 20 in the first embodiment, and includes a substrate 52, a first electrode 54, a second electrode 54', and two line-shaped carbon nanotube elements 56. The first electrode 54 and the second electrode 54' are parallel to each other and disposed on the substrate 52.

The two carbon nanotube elements 56 are respectively fixed on the first electrode 54 and the second electrode 54'. A groove 58 is formed on the surface of the substrate 52 between the first electrode 54 and the second electrode 54'. Due to the insulative nature of the substrate 52, a shield effect against the emitted electrons may occur. The groove 58 can increase the distance between the carbon nanotube element 56 and the substrate 52. Accordingly, the shield effect can be reduced.

Referring to FIG. 8, the surface-conduction electron emitter 60 in the fourth embodiment is similar to the surface-conduction electron emitter 20 in the first embodiment, and includes a substrate 62, a first electrode 64, a second electrode 64', and two carbon nanotube elements 66. The first electrode 64 and the second electrode 64' are parallel to each other and disposed on the substrate 62.

The two carbon nanotube elements 66 are fixed on the first electrode 64 and the second electrode 64' respectively. Two fixing layers 68 are disposed on the first electrode 64 and the second electrode 64' respectively. The protruding part of the carbon nanotube elements 66 and the top surface of the first electrode 64 and the second electrode 64' are covered by the fixing layers 68. The fixing layers 68 can, usefully, be made of an insulative material selected from a group consisting of silicon dioxide, silicon nitride, metal oxides, ceramic and photoresist. The fixing layers 68 can enhance the stability of the carbon nanotube elements 66 and prevent a draw-out effect thereof caused by the electrical field.

Additionally, it is to be understood that a tooth-shaped structure can be further formed on the emitting ends of the carbon nanotube elements, as shown in FIG. 9, to prevent the shield effect caused by the adjacent carbon nanotube ele-

ments 26 of the first electrode 24 or the second electrode 24'. Thus, the emitting property of the carbon nanotube elements 26 can be enhanced.

Referring to FIG. 10 to FIG. 14, a method for fabricating the surface-conduction electron emitter 20 includes the steps of: (a) providing a substrate 22; (b) disposing two lower layers 242 and 242' on the surface of the substrate 22, the two lower layers 242 and 242' are parallel and apart from each other; (c) disposing a plurality of carbon nanotube elements 26 on the lower layers 242 and 242'; (d) disposing two upper layers 244 and 244' on the two lower layers 242 and 242', and thereby, sandwiching the carbon nanotube elements 26; and (e) forming a micro-fissure 28 between the carbon nanotube elements 26.

In step (a), the substrate 22 can, beneficially, be made of an insulative material selected from a group consisting of quartz, glass, ceramic, and plastic, or of a conductive material with an insulative layer formed thereon. The insulative layer can, usefully, be an oxide layer. The thickness of the substrate 22 is dependent on the actual needs/use. In the present embodiment, the substrate 22 is made of a silicon wafer with a silicon dioxide layer formed thereon. The thickness of the silicon dioxide layer is in the approximate range from 0.5 to 1 micron.

Referring to FIG. 11, in step (b), the two lower layer 242 and 242' can be formed by either a lift-off step or an etching step of photolithography.

In the lift-off step, a photoresist layer is disposed on the surface of the substrate 22. Two parallel sections of the photoresist layer are removed. Accordingly, the substrate 22 is exposed at the two parallel sections. Then, a metallic layer or a plurality of metallic layers is deposited on the substrate 22 by means of vacuum evaporation, magnetron sputtering, or electron beam evaporation. After the metallic layer has been deposited, the substrate 22 is immersed in an organic solvent to remove the photoresist layer and the metallic layer formed thereon. Thereby, the two lower layers 242 and 242' are formed on the substrate 22. Quite suitably, the organic solvent is acetone.

In the etching step, a metallic layer or a plurality of metallic layers are deposit on the substrate 22. The photoresist layer is formed on the metallic layer. Then the photoresist layer is removed except for two parallel sections. Further, the exposed substrate 22 is etched by means of chemical wet etching or reactive ion etching. Finally, the substrate is immersed in an organic solvent to remove the photoresist layer, and thereby, to achieve the two lower layers 242 and 242'. Quite suitably, the organic solvent is acetone.

The two lower layers can, opportunely, be made of a metallic material such as titanium (Ti), platinum (Pt), tungsten (W), palladium (Pd), or gold. The thickness of the two lower layers is in the approximate range from 40 to 70 nanometers. The length and the width are both in the approximate range from several tens of microns to several hundreds of microns. The distance between the two lower layers is in the approximate range from several microns to several tens of microns. Quite suitably, the lower layers 242 and 242' can be made of a metallic material with a high friction coefficient such as titanium (Ti) or tungsten (W) to enhance the friction between the lower layers 242 and 242' and the substrate 22.

Furthermore, the lower layers 242 and 242' can include a plurality of metallic layers. The lower layer contacted with the substrate 22 can, suitably, be made of a metallic material with high friction coefficient such as titanium (Ti) or tungsten (W). The upper layer contacted with the carbon nanotube elements 26 can, beneficially, be made of a metallic material with high conductivity such as gold, platinum (Pt) or palla-

dium (Pd) to enhance the electrical contact and reduce the contact resistance between the lower layers 242 and 242' and the carbon nanotube elements 26.

In step (c), referring to FIG. 12, a plurality of the carbon nanotube elements 26 can be adhered, sprayed or deposited on the lower layers 242 and 242'. The carbon nanotube elements 26 are parallel to each other and the substrate 22. The carbon nanotube element 26 can, advantageously, include at least one material selected from a group consisting of carbon nanotubes and carbon nanotube bundles.

In step (c), the carbon nanotube elements can be adhered on the lower layers 242 and 242' by the substeps of: (c1) providing a carbon nanotube film; (c2) adhering the carbon nanotube film on the top of the lower layers 242 and 242'; and (c3) soaking the carbon nanotube film in an organic solvent (e.g. ethanol).

In step (c1), the carbon nanotube film can, usefully, be fabricated by pulling out a plurality of carbon nanotube segments from an array of carbon nanotubes by using a tool (e.g., adhesive tape, a tweezers, or other tools allowing multiple carbon nanotubes to be gripped and pulled simultaneously). Quite suitably, the array of carbon nanotubes is a super-aligned array of carbon nanotubes. During the pulling process, the carbon nanotube segments can be pulled out end to end, due to the van der Waals attractive force between ends of the adjacent carbon nanotube segments, to form a successive carbon nanotube film (Xiaobo Zhang et al., Advanced Materials, 18, 1505 (2006)).

It is to be understood that an adhesive/glue can be directly applied on an edge of the substrate 22 with lower layers 242 and 242' formed thereon. The edge of the substrate 22 with the adhesive/glue is attached to the array of carbon nanotubes. Then the substrate 22 is moved along the direction from the one lower layer 242 to the other lower layers 242'. As such, a carbon nanotube film can be pulled out and adhered to the lower layers 242 and 242'. Finally, the carbon nanotube film as above described is soaked in an organic solvent.

In step (c), the carbon nanotube elements can be sprayed on the lower layers 242 and 242' by the substeps of: (c1') dispersing a plurality of carbon nanotubes in a solvent; (c2') spraying the solvent, with a plurality of carbon nanotubes dispersed therein, on the lower layers 242 and 242'; and (c3') volatilizing the solvent, in order to achieve a plurality of carbon nanotubes disposed on the lower layers 242 and 242'.

In step (c1'), the solvent can, beneficially, be a volatilizable organic solvent and can be selected from the group consisting of ethanol, acetone, dichloroethane, isopropanol, and combinations thereof. In another embodiment, the solvent can also be a surfactant solution (e.g. a solution of sodium dodecyl benzene sulfonate (SDBS)). In step (c2'), the lower layers 242 and 242' can, opportunely, be heated to the boiling point before sprayed by the solvent. As such, the solvent can volatilize quickly at high temperature to keep carbon nanotubes from aggregating on the lower layers 242 and 242'.

Quite usefully, an additional step (c4) of orienting the carbon nanotubes on the lower layers 242 and 242' can, advantageously, be further provided after the step (c3'). The orientation of carbon nanotubes can be formed by an electro-phoretic method or an airflow method. The orientation of the carbon nanotubes is along the direction from one lower layer 242 toward the other lower layer 242'.

In step (c), the carbon nanotube elements can be deposited on the lower layers 242 and 242' by the substeps of: (c1") dispersing a plurality of carbon nanotubes in a solvent; (c2") immersing the substrate 22, with the lower layers 242 and 242' formed thereon, in the solvent with the carbon nanotubes dispersed therein; and (c3") standing for a period of time (e.g.

several hours), volatilizing the solvent completely, in order to achieve a plurality of carbon nanotubes disposed on the lower layers 242 and 242'.

In step (c1"), the solvent can, beneficially, be a volatilizable organic solvent and can be selected from the group consisting of ethanol, acetone, dichloroethane, isopropanol, and combinations thereof. In another embodiment, the solvent can also be a surfactant solution (e.g. a solution of sodium dodecyl benzene sulfonate (SDBS)). In step (c2"), the carbon nanotubes deposit on the lower layers 242 and 242' under force of gravity.

Quite usefully, an additional step (c4") of orienting the carbon nanotubes on the lower layers 242 and 242' can, advantageously, be further provided after the step (c3"). The orientation of carbon nanotubes can be formed by an electro-phoretic method or an airflow method. The orientation of the carbon nanotubes is along the direction from one lower layer 242 toward the other lower layer 242'.

In step (d), referring to FIG. 13, the step of forming the two upper layers 244 and 244' is similar to step (b) of forming the two lower layers 242 and 242'. The material of the two upper layers can, opportunely, be a metallic material such as titanium (Ti), platinum (Pt), tungsten (W), palladium (Pd), or gold. Quite suitably, the two upper layers can be made of a metallic material with high conductivity such as palladium (Pd), or gold.

In step (e), referring to FIG. 14, the micro-fissure 28 can be formed between the carbon nanotube elements 26 by the substeps of: (e1) forming a photoresist layer on the carbon nanotube elements 26 and the surface of the upper layers 244 and 244'; (e2) exposing a section of the carbon nanotube elements from the photoresist layer by a photolithography method; and (e3) removing the exposed section of the carbon nanotube elements by means of plasma etching, and forming a micro-fissure 28 between the carbon nanotube elements 26.

The width of the micro-fissure can, opportunely, be in the approximate range from 1 to 10 microns. In step (e3), the gas used in plasma etching can be selected from a group consisting of hydrogen, oxygen, sulfur hexafluoride, and any combination thereof. In the present embodiment, the gas used in plasma etching is oxygen, the pressure is about 2 Pascal (Pa), the power is about 100 Watt (W), and the time of etching is about 2 minutes.

In step (c), an excess of carbon nanotubes may be disposed on the substrate 22. Therefore, in step (e), the excess carbon nanotubes can be removed by plasma etching.

The method for fabricating the surface-conduction electron emitter 40 in the second embodiment is similar to the method for fabricating the surface-conduction electron emitter 20 in the first embodiment. In the method for fabricating the surface-conduction electron emitter 40, an additional step of forming a spacer 48 on the surface of the substrate 42 between the lower layers 442 and 442' is further provided before step (c).

The spacer 48 can, suitably, be formed by means of vacuum evaporation, magnetron sputtering, or electron beam evaporation. The spacer 48 can, beneficially, be made of a material selected from a group consisting of silicon dioxide, alumina, metal oxides, and ceramic. The thickness of the spacer 48 is less than or equal to the thickness of the lower layers 442 and 442'. In the second embodiment, the spacer is a silicon dioxide layer. The thickness of the spacer is in the approximate range from 40 to 70 nanometers.

The method for fabricating the surface-conduction electron emitter 50 in the third embodiment is similar to the method for fabricating the surface-conduction electron emitter 20 in the first embodiment. In the method for fabricating

the surface-conduction electron emitter **50**, an additional step of forming a groove **58** on the surface of the substrate **52** between the first electrode **54** and the second electrode **54'** is further provided after step (e).

The groove **58** can, beneficially, be formed by means of chemical wet etching. Due to the insulative nature of the substrate **52**, a shield effect against the emitted electrons may be occurred by the substrate **52**. The groove **58** can increase the distance between the carbon nanotube element **56** and the substrate **52**. Accordingly, the shield effect can be reduced. The etchant used in chemical wet etching is dependent on the material of the substrate **52**. In the present embodiment, the substrate **52** is a silicon wafer with a layer of silicon dioxide formed thereon, the etchant, therefore, is a solution of sodium hydroxide at about 80° C., the etching time is about 10 minutes, and the depth of the groove **58** is in the approximate range from 10 microns to 20 microns.

The method for fabricating the surface-conduction electron emitter **60** in the fourth embodiment is similar to the method for fabricating the surface-conduction electron emitter **20** in the first embodiment. In the method for fabricating the surface-conduction electron emitter **60**, the photoresist layer on the first electrode **64** and the second electrode **64'** and the carbon nanotube elements **66** protruding from the first electrode **64** and the second electrode **64'** are preserved after step (e) to be used as the fixing layers **68**. The fixing layers **68** can enhance the stability of the carbon nanotube elements **66** and prevent a draw-out effect thereof caused by the electrical field. In another embodiment, the fixing layers **68** can be further formed by a depositing step after step (d). The fixing layers **68** can, usefully, be made of an insulative material selected from a group consisting of silicon dioxide, silicon nitride, metal oxides, and ceramic.

Additionally, in step (e), a tooth-shaped structure can be further formed on the carbon nanotube elements protruding from the electrodes by using a tooth-shaped photolithography mask. Accordingly, a tooth-shaped micro-fissure can be formed between the carbon nanotube elements. Referring to FIG. 9, the tooth-shaped structure can prevent the shield effect caused by the adjacent carbon nanotube elements **26** of the first electrode **24** or the second electrode **24'**. Thus, the emitting property of the carbon nanotube elements **26** can be enhanced. It is to be understood that the shape of the structure of the carbon nanotube elements is arbitrary and other shapes can be formed by the same method.

A method for fabricating the electron source **30** is similar to the method for fabricating the surface-conduction electron emitter **20** and includes the steps of: (a') providing a substrate **22**; (b') disposing a plurality of lower layers on the surface of the substrate **22**; (c') disposing a plurality of carbon nanotube elements **26** on the lower layers; (d') disposing a plurality of upper layers on the lower layers, thereby, sandwiching the carbon nanotube elements; and (e') forming a plurality of micro-fissures **28** between the carbon nanotube elements **26**.

The lower layers are parallel to each other and in the same shape as the upper layers. The carbon nanotube elements **26** are parallel to each other.

The surface-conduction electron emitters and the electron sources using the same in the present embodiments can be simply fabricated by means of photolithography and deposition. Therefore, the cost of the fabrication is reduced. Further, the width of the micro-fissures is about several microns. The electrons emitted from the carbon nanotube elements can be effectively deviated to collide with the fluorescent layer. As such, the efficiency of the electron sources is relatively high. Additionally, due to the excellent field emission property of the carbon nanotubes, the voltage needing to be applied on the electrodes is reduced. Thus, the energy consumption of the electron emitters is reduced.

Finally, it is to be understood that the above-described embodiments are intended to illustrate rather than limit the invention. Variations may be made to the embodiments without departing from the spirit of the invention as claimed. The above-described embodiments illustrate the scope of the invention but do not restrict the scope of the invention.

The invention claimed is:

1. A method for fabricating a surface-conduction electron emitter, the method comprising the steps of:

- (a) providing a substrate comprising a surface;
- (b) disposing a first lower electrode layer and a second lower electrode layer on the surface of the substrate, the first lower electrode layer and second lower electrode layer are parallel and apart from each other;
- (c) disposing a plurality of carbon nanotube elements on the first lower electrode layer and the second lower electrode layer;
- (d) disposing a first upper electrode layer on the first lower electrode layer, and disposing a second upper electrode layer on the second lower electrode layer; wherein a portion of the plurality of carbon nanotube elements are in contact with and sandwiched between the first lower electrode layer and the first upper electrode layer and another portion of the plurality of carbon nanotube elements are in contact with and sandwiched between the second lower electrode layer and the second upper electrode layer; and
- (e) forming a micro-fissure between the carbon nanotube elements.

2. The method as claimed in claim 1, wherein the first and second lower electrode layers, and the first and second upper electrode layers are formed by means of vacuum evaporation, magnetron sputtering, or electron beam evaporation.

3. The method as claimed in claim 1, wherein the carbon nanotube elements are carbon nanotube bundles adhered, on the first and second lower electrode layers, and each of the carbon nanotube bundles comprises of a plurality of carbon nanotubes joined end to end.

4. The method as claimed in claim 3, wherein the carbon nanotube elements are adhered to the first and second lower electrode layers by the substeps of:

- (c1) pulling out a plurality of carbon nanotube segments end to end from an array of carbon nanotubes by using a tool to form a carbon nanotube film;
- (c2) adhering the carbon nanotube film on a top of the first and second lower electrode layers; and
- (c3) soaking the carbon nanotube film with an organic solvent to form a plurality of carbon nanotube bundles shrunk from the carbon nanotube film.

5. The method as claimed in claim 4, wherein the tool allows multiple carbon nanotubes to be gripped and pulled simultaneously, the carbon nanotube segments are pulled out end to end due to the van der Waals attractive force between ends of the adjacent carbon nanotube segments, to form the carbon nanotube film.

6. The method as claimed in claim 4, wherein the carbon nanotube elements are parallel to each other and parallel to the surface of the substrate; each of the carbon nanotube elements comprises a first and a second emitting end, and the first emitting end is located between the first upper and lower electrode layers, and the second emitting end is located between the second upper and lower electrode layers, thereby forming the micro-fissure therebetween.

7. The method as claimed in claim 3, wherein the carbon nanotube elements are adhered to the first lower electrode layer and the second lower electrode layer by the substeps of:

## 11

applying an adhesive on the substrate with the first lower electrode layer and the second lower electrode layer formed thereon;

attaching the adhesive on the substrate to an array of carbon nanotubes;

moving the substrate along a direction from the first lower electrode layer the second lower electrode layer to pull out a carbon nanotube film from the array of carbon nanotubes and adhere the carbon nanotube film to the first lower electrode layer and second lower electrode layer; and

soaking the carbon nanotube film with an organic solvent to form the carbon nanotube bundles shrunk from the carbon nanotube film.

8. The method as claimed in claim 1, wherein the carbon nanotube elements are sprayed on the first and second lower electrode layers by the substeps of:

(c1') dispersing a plurality of carbon nanotubes in a solvent;

(c2') spraying the solvent, with a plurality of carbon nanotubes dispersed therein, on the first lower electrode layer and the second lower electrode layer; and

(c3') volatilizing the solvent, in order to achieve a plurality of carbon nanotubes disposed on the first lower electrode layer and the second lower electrode layer.

9. The method as claimed in claim 8, further comprising orienting the carbon nanotubes along a direction from the first lower electrode layer to the second lower electrode layer.

10. The method as claimed in claim 1, wherein the carbon nanotube elements are deposited on the first lower electrode layer and the second lower electrode layer by the substeps of:

(c1'') dispersing a plurality of carbon nanotubes in a solvent;

(c2'') immersing the substrate, with the first lower electrode layer and the second lower electrode layer formed thereon, in the solvent with the carbon nanotubes dispersed therein; and

(c3'') standing for a period of time, volatilizing the solvent completely, in order to achieve a plurality of carbon nanotubes disposed on the first lower electrode layer and the second lower electrode layer.

11. The method as claimed in claim 10, wherein an additional step of orienting the carbon nanotubes along a direction from the first lower electrode layer to the second lower electrode layer is further provided.

12. The method as claimed in claim 1, wherein the microfissure is formed between the carbon nanotube elements by the substeps of:

(e1) forming a photoresist layer on the carbon nanotube elements and the first upper electrode layer and the second upper electrode layer;

(e2) exposing a section of the carbon nanotube elements between the first upper electrode layer and the second upper electrode layer through the photoresist layer by a photolithography method; and

(e3) removing the exposed section of the carbon nanotube elements by means of plasma etching, and forming the microfissure between the first upper electrode layer and the second upper electrode layer.

13. The method as claimed in claim 12, wherein the photoresist layer on the first upper electrode layer and the second upper electrode layer and the carbon nanotube elements are preserved after step (e3) to be used as fixing layers.

14. The method as claimed in claim 12, wherein a tooth-shaped microfissure is further formed between the carbon nanotube elements by using a tooth-shaped photolithography mask.

## 12

15. The method as claimed in claim 1, wherein an additional step of forming fixing layers on a top surface of the first upper electrode layer, the second upper electrode layer and the carbon nanotube elements is further provided before step (e).

16. The method as claimed in claim 1, wherein an additional step of forming a spacer on the surface of the substrate between the first lower electrode layer and the second lower electrode layer is further provided before step (c), a thickness of the spacer is less than or equal to a thickness of the first lower electrode layer and the second lower electrode layer.

17. The method as claimed in claim 1, further comprising of a first electrode and a second electrode; wherein the first electrode comprises of the first lower electrode layer and the first upper electrode layer, and the second electrode comprises of the second lower electrode layer and the second upper electrode layer.

18. The method as claimed in claim 17, further comprising, after step (e), forming a groove on the surface of the substrate between the first electrode and the second electrode to increase a distance between the carbon nanotube elements and the substrate to reduce a shielding effect.

19. A method for fabricating a surface-conduction electron source, the method comprising the steps of:

(a') providing a substrate comprising a surface;

(b') disposing a plurality of lower electrode layers on the surface of the substrate;

(c') disposing a plurality of carbon nanotube elements on top surfaces of the lower electrode layers;

(d') disposing a plurality of upper electrode layers on the top surfaces of the lower electrode layers, thereby, sandwiching and electrically connecting the carbon nanotube elements between each of the lower electrode layers and each of the upper electrode layers; and

(e') forming a plurality of micro-fissures between the carbon nanotube elements.

20. A method for fabricating a surface-conduction electron emitter, the method comprising the steps of:

(a) providing a substrate;

(b) disposing a first lower electrode layer and a second lower electrode layer apart from each other on the substrate;

(c) drawing a carbon nanotube film from an array of carbon nanotubes, the carbon nanotube film consisting of carbon nanotubes;

(d) adhering the carbon nanotube film on a top surface of the first lower electrode layer and a top surface of the second lower electrode layer;

(e) disposing a first upper electrode layer on the top surface of first lower electrode layer, and disposing a second upper electrode layer on the top surface of the second lower electrode layer; wherein a portion of the carbon nanotube film is sandwiched between and electrically connected to the first lower electrode layer and the first upper electrode layer and another portion of the carbon nanotube film is sandwiched between and electrically connected to the second lower electrode layer and the second upper electrode layer;

(f) soaking the carbon nanotube film with an organic solvent to form a plurality of carbon nanotube bundles shrunk from the carbon nanotube film; and

(g) forming a micro-fissure in the carbon nanotube bundles located between the first lower electrode layer and the second lower electrode layer.